# EUROPEAN PATENT SPECIFICATION

(11) **EP 1 432 085 B1**
(45) Date of publication and mention of the grant of the patent: **17.09.2008**
(21) Application number: 02394117.2
(22) Date of filing: 19.12.2002
(51) Int. Cl.: H01R 39/24

(54) **Carbon fiber electrical contacts formed of composite carbon fiber material**
Elektrische Kohlenstofffaserkontakte aus Kohlenstofffaserverbundmaterial
Contacts èlectriques en fibre de carbone formès avec du matériel en fibre de carbone composite

(43) Date of publication of application: 23.06.2004
(73) Proprietor: Micro Contacts Inc, Hicksville, New York 11801 (US)
(72) Inventor: Tucci, Michael, c/o Micro Contacts Inc., Hicksville, New York 11801 (US); Uruburu, Philip, c/o Micro Contacts Inc., Hicksville, New York 11801 (US); Veselaski, Stephen, c/o Micro Contacts Inc., Hicksville, New York 11801 (US)
(74) Representative: Coyle, Philip Aidan

(56) References cited:
- US-A- 4 460 633
- US-A1- 2003 008 125
- US-B1- 6 444 102

## Description

This invention relates generally to an electrical contact or an electrical contact assembly typically used in an electromechanical device and, more particularly, to a contact or contact assembly, which is formed of a composite material using carbon fibers and a nonwoven carbon fiber mat, as the element that makes electrical contact with another element of the electromechanical device.

Variable resistive devices utilize elements that vary a voltage or current in order to provide an electrical signal that indicates a relationship to a physical position of a contact or wiper on a resistive or conductive element. Because these variable resistive devices are used in a dynamic state they can not be fixed or restricted in their movement and must have the freedom to be positioned along any length of their respective resistive or conductive paths. The contact or wiper must therefore be produced of a material that is electrically, physically, and environmentally compatible with the resistive and/or conductive track when in the presence of an electrically active and physically dynamic system. The contact or wiper must also provide a long useful life, while maintaining uniform positive engagement with the resistive or conductive element and not produce polymers or debris which act as an insulator and distorts the output signal.

Presently the contact or wiper materials used for these variable resistive devices are composed of various clad or coated metals or precious metal alloys. These precious metal containing contacts, in a dynamic state and in the presence of electrical activity, act as catalysts to generate polymers and debris which degrade the resistive track output signals. This results in the early termination of accurate performance and useful life.

Initially metal contacts or wipers were used with wirewound resistive or metallic conductive elements, because wirewound elements were the most precise devices. As time evolved great improvements were made in the non-wirewound product area, and they supplanted the wirewound resistive element, but the contact or wiper has always created problems relative to the resistive element because in the presence of an electrical current and dynamic performance, the precious metal components of the metallic contact provide the catalyst to generate polymers and debris, which interfere with the accuracy of the output signal.

Now that reduction in size, improved accuracy, and a reduction in electrical contact resistance are required in modem servo feed-back positioning systems, non-metallic contact materials must be considered to obtain the necessary and sorely needed improvements in these performance characteristics and elimination of the polymers and debris.

US 6,444,102 discloses an electrical contact according to the pre-characterizing portion of claim 1.

The need exists for improvements in electrical contacts and contact assemblies and, particularly, for-improvements in the materials and assemblies employed therefor.

Accordingly, it is an object of the present invention to provide a contact or contact assembly for use in electromechanical applications that can effectively eliminate the above-noted defects inherent in previously proposed systems.

It is another object of this invention to eliminate the above-described negative conditions and characteristics of previously known systems and to improve considerably the useful life of the system by providing a contact or wiper formed of nonmetallic material, such as one formed of a composite carbon fiber material including carbon fibers and a nonwoven carbon filter mat. This composite carbon fiber material, through special processing, not only overcomes the negative conditions caused by metal composition contacts or wipers, but considerably improves total performance in all other aspects.

It is a further object of the present invention to provide a wiper contact or contact assembly for use in electromechanical components or applications that is more compatible with present state of the art fabrication techniques and materials used for resistive and conductive track substrates and that appreciably reduces or eliminates the negative aspects inherent in presently used or previously proposed designs or materials.

According to the present invention there is provided an electrical contact characterised according to claim 1.

In a preferred embodiment, an existing contact carrier is employed and in place of the previously used metal contacts, and the contacts are specially attached to the carrier.

In a preferred embodiment, the contact is processed and formed in such a manner as to allow-the multiple strands of carbon fiber at the center layer of the composite material when properly positioned to be electrically conductive for transmitting umimpeded electrical signals along their longitudinal length. Such carbon fiber strands may be fused or conductively bonded by any of various techniques to provide essentially uniform conductivity and redundant transmission of the electrical signal. Additional, off-axis electrical conductivity is provided by nonwoven carbon fiber mats placed on the sides of the multiple strands of carbon fiber. The composite carbon fiber material can be affixed to a carrier or the material may be utilized without a carrier. Such a carrier, if used, may be metallic or non-metallic and may be affixed to the composite carbon fiber material by any of various bonding, fusing, and fastening techniques. The carrier can also be electrically nonconductive, depending upon the application. Alternatively, the carrier can be formed of the same homogenous composite carbon fiber material as that used for the actual contact. Forming of the carbon fiber contact layer of the composite material can involve cross-layering of the material in nonparallel orientations to provide additional structural integrity, as well as to assist in the post-forming operation.

The contact can be rigid enough to sustain and maintain a consistent position relative to its parallel alignment to the resistive or conductive track of the substrate element and yet be flexible enough in a perpendicular position to the track to allow some variation in movement to sustain uniform contact position, spring rate and pressure. Thus, the electrical output signal maintains its integrity.

In a further preferred embodiment, the contact surface of the wiper contact that is adjacent to the resistive or conductive track is composed of multiple points of contact, rather than either a small number of metal fibers or just one broad band of a rigid beam contact. This ensures a more redundant positive footprint with the resistive or conductive track, which reduces contact resistance and variable electrical noise.

Embodiments of the invention will now be described, by way of example, with reference to the accompanying drawings, in which:
Figs. 1A-1D are side elevations showing respective embodiments of electrical contacts according to the present invention;
Figs. 2A-2C are front elevations and respective enlargements showing embodiments of electrical contacts corresponding to Figs. 1A-1C, respectively;
Fig. 3 shows two views of a carbon fiber contact formed as a matrix of layers of carbon fibers;
Fig. 4 shows two views of a carbon fiber contact formed as a matrix of layers of carbon fibers;
Fig. 5 shows two views of an electrical contact formed solely of carbon fibers according to an embodiment of the present invention;
Fig. 6 shows two views of an electrical contact formed solely of carbon fibers according to another embodiment of the present invention;
Fig. 7 shows two views of a carbon fiber electrical contact affixed to an electrically conductive beam according to an embodiment of the present invention;
Fig. 8 shows two views of an electrical contact in which the carbon fibers are mechanically captured and chemically fused accordingly to an embodiment of the present invention;
Fig. 9 shows two views of an electrical contact in which the carbon fibers are mechanically captured and chemically fused according to an embodiment of the present invention;
Fig. 10 shows two views of an electrical contact in which the carbon fibers are mechanically captured and chemically fused accordingly to an embodiment of the present invention;
Fig. 11 shows two views of an electrical contact employing multiple layers on a carrier according to an embodiment of the present invention;
Fig. 12 shows two views of an electrical contact formed as a single carbon fiber element;
Fig. 13 is an exploded view showing the carbon fibers in juxtaposition with two carbon fiber nonwoven mats; and
Fig. 14 is an end view showing the several layers making up an embodiment of the inventive composite carbon fiber material.

The present invention provides a contact or wiper element for transmitting electrical signals, either in a low voltage mode (under 15 volts) or a low current mode (under 500 ma) between a resistive and/or a conductive track and some external circuit termination. In one embodiment-the contact or wiper element comprises one or more thin, single layers of carbon fiber elements, all aligned in one direction bonded together and firmly fixed in a very low-resistance, synthetic resin compound for structural stability and electrical continuity and which form part of a composite carbon fiber material described below.

Although in the following description of several embodiments of the inventive electrical contact various forms of the carbon fiber bundles or strands are described, it is to be understood that the electrical contacts are formed of the composite carbon fiber material described below in relation to Figs. 13 and 14.

As shown in Figs. 1A-1C, the ends of the contact or wiper may be specially formed to give the engagement portion of the contact or wiper added strength and permit better mating of the carbon fiber element to the track of the device. In Fig. 1A, the contact 10 has a rake end 12. In Fig. 1B, the contact 14 has a knuckle end 16. In Fig. 1C, the contact 18 has a pointed end 20.

The contact or wiper 22, as shown in Fig. 1D, may also engage a mechanical strip 24 for support or for attachment purposes. The mechanical strip 24 may be electrically conductive or not, depending upon the desired application.

Figs. 2A, 2B, and 2C correspond, respectively, to Figs. 1A, 1B. and 1C and show the arrangement of the carbon fiber bundles that are part of the composite material forming the specialized end constructions 12, 16, and 20, respectively. That is, the enlargement of Fig. 2A shows carbon fiber bundles 26 arranged in one layer forming the rake end 12. Similarly, bundles 28 and 30 respectively form knuckle end 16 and pointed end 20 in Figs. 2B and 2C, respectively. The other layers of the composite material are not shown because the structures of the carbon fiber bundles would be obscured.

In the embodiment shown in Fig. 3, the contact or wiper element 40 is formed of a carbon fiber matrix, whose adjacent three carbon fiber layers 42, 44, 46 are essentially perpendicular to each other. The carbon fibers forming layers 42, 44, 46 are not bundled but are discretely placed-in a cross-hatching matrix, wherein the fibers in alternate layers may be parallel to each other, but those in adjacent layers are essentially nonparallel and may be perpendicular to each other.

Fig. 4 shows a similarly constructed contact 50 in which the carbon fibers of only one layer 52 perform the actual contacting and an inner layer 54 and second outer layer provide structural support. The additional layers of the composite material are shown in Fig. 14.

The matrix composition shown in the embodiments of Figs. 3 and 4 reinforces and strengthens the minuscule carbon fiber strands to provide support for retaining stable contact position. The carbon fiber strands may be continuous or discontinuous and the matrix need not necessarily be homogeneous.

Corresponding to the structure shown in Fig. 1D, the matrix compositions of Figs. 3 and 4 can use an additional mechanical support strip, which can be electrically conductive depending upon the desired application. The carbon fibers of the matrix composition shown in Figs. 3 and 4 are firmly fixed in a very low resistance synthetic resin compound to restrict movement, add structural stability, and provide multidirectional electrical continuity.

As shown in Fig. 5, the planar form of a carbon fiber contact element 60 can consist of a single layer, not a matrix of carbon fiber strands, arranged in a horseshoe shape or upside-down U to provide a continuous, unbroken path from one end 62 of the carbon fiber element strands, one of which is shown typically at 64, to the other end 66, even though the carbon fiber strands may change direction by more than 90 degrees. In this embodiment each carbon fiber strand 64 will be both perpendicular and parallel to the resistive or conductive track, not shown, and each opposing end 62,66 of the continuous carbon fiber strands 64 will essentially contact different parallel resistive or conductive tracks, not shown. The horseshoe shaped contact 60 can employ a carrier, not shown, which can be electrically conductive or not, depending on the desired application.

A similar construction is shown in Fig. 6, wherein the contact 70 has a right-angle transition portion 72 in the path from one end 74 to the other end 76.

In the embodiment shown in Fig. 7, a contact assembly 80 has a carbon fiber element formed as a very short strip 82 firmly and conductively attached at 84 by a conductive adhesive to a parallel portion 84 of a thin beam 86 composed of electrically conductive material. This beam construction provides a means for the current or voltage signal to flow unimpeded from the resistive or conductive track to the end terminus, thereby incorporating the compatible and desirable characteristics of the carbon fiber contact material with beam members formed of materials other than carbon fiber. When this embodiment is in use, the carbon fiber element 82 will be essentially perpendicular to the plane of the resistive or conductive track at all times.

In the embodiment of the present invention shown in Figs. 2A, 2B, and 2C, the planar form of the carbon fiber element consists of one or more parallel layers of carbon fiber strip arranged so that the free ends 12, 16, 20 of the carbon fiber elements 10, 14, 18, respectively, are designated as the ends that will contact the tracks of the resistive element or conductive element. It is a feature of the present invention that those ends 12, 16, 20 can be fabricated free of any other material, such as the low-resistance, synthetic resin compound or the like, for a length less than 3/16' (4.7625mm) to permit only the actual carbon fiber material to contact the respective tracks, thereby providing improved mating between the ends 12, 16, 20 of the contacts 10, 14, 18 and the tracks, not shown, of the respective conductive elements. The free end of the contact may remain parallel in the same plane or, as shown in Figs. 2A, 2B, and 2C, the free end may be bent or formed to an angle perpendicular to the primary length of the strip or formed into a knuckle shape depending upon the application.

In the embodiments shown in Figs. 8, 9, and 10, each contact or wiper element 90, 92, 94, respectively, is fabricated in narrow strips of carbon fiber element, one of which is shown at 96, 98, 100, respectively, wherein each strip is less than 0.015'(0.3810mm) in width and is composed or one or more parallel strands of carbon fibers. A number of these strips are arranged in a single flat plane, with each strip being essentially parallel to, but not fused or chemically bonded to, each other. The multiple independent parallel strips are mechanically captured by respective collars 102, 104, 106, in a single plane and/or chemically bonded with a low-resistance, electrically conductive synthetic resin compound at one end of the assembled strips, so that the independent multiple strip sections will be electrically uniform in their output signal and also be receptive to further assembly operations.

As shown in Figs. 8, 9, and 10, the free ends 108, 110, 112 of the respective multiple strip sections 90, 92, 94 that are to function as the intimate contact points with the track of the resistive or conductive element can remain coplanar to the strip or be formed as a rake as shown in Fig. 8, a knuckle as shown in Fig. 9, or other compatible contact geometry, such as the point as shown in Fig. 10. This feature permits the assembly to contain multiple contact strips, such as 96, 98, 100, each with relatively independent mechanical movement in a direction perpendicular to the resistive or conductive track of the substrate element.

Fig. 11 is an embodiment similar to that of Fig. 7 wherein multiple layers 120, 122, 124, of carbon fiber elements are attached to a shorter leg 126 of an L-shaped carrier 128. The carbon fibers in each layer 120, 122, 124 are substantially aligned to be parallel and the layers may be attached to the carrier by an electrically conductive synthetic resin compound shown generally at 130.

As shown in the embodiments of Figs. 3, 4, and 11, the electrical contact devices are formed of multiple layers of carbon fibers in various alignments, Similarly, all other embodiments herein shown and described can be formed of multiple layers. So too, the various embodiments of the present invention can be used with a carrier that can be electrically conductive or not, depending upon the desired application.

Conversely, as shown in Fig. 12, an electrical contact or wiper 140 can be formed of only a single carbon fiber element 142 that can be around 0.010' to 0.015' (0.2540 to 0.3810mm) in thickness. Although a rake end 144 is provided in this embodiment, any of the other end treatments described above are also appropriate.

As noted hereinabove, all of the embodiments described so far can be formed from a composite carbon fiber material that has as its core a carbon fiber structure that has carbon fiber bundles arranged in one layer, as in Figs. 2A-2C, or in multiple layers, as in Fig. 3.

As shown in Fig. 13, a layer of the carbon fiber bundles 150 has mats 152, 154 formed of nonwoven carbon fibers arranged on each flat side. Although not shown in Fig. 13, following the placement of the mats 152, 154 on the carbon fiber bundle structure 150, a thermoplastic resin is applied to the exterior surfaces of the mats 152, 154. This thermoplastic resin, or polymer, completes the structure and bonds the mats 152, 154 to the carbon fiber bundle structure 150, thereby forming a stable composite material. The nonwoven carbon-fiber mat 152 or 154 is substantially isotropic and the fibers are so randomly arranged as to provide little or no directionality in the plane of the mat.

The nonwoven carbon fiber mat provides a primary electrical current carrying capacity and also provides improved mechanical strength to the overall construction. More specifically, the nonwoven carbon fiber provides off-axis mechanical stability, as well as off-axis current carrying capability, where the off-axis term relates to a longitudinal direction of the finally manufactured electrical contact.

The nonwoven carbon fiber mat is available commercially from Hollingsworth & Vose Company, East Walpole, Massachusetts and ranges in thickness from 0.08 mm to 0.79 **mm.**

Fig. 14 is an end view of the assembled composite material 160 described above in which the nonwoven carbon fiber mats 152, 154 are arranged on the carbon fiber structure 150 and in which thermoplastic resin layer 162 is applied over the nonwoven carbon fiber layer 152 and a thermoplastic resin layer 164 is applied over the nonwoven carbon fiber mat 154. This results in a stable composite material that can be formed to any desired shape, as described and shown in regard to the several embodiments shown herein.

## Claims

1. An electrical device for transmitting electrical signals and for movable contact with an electrically conductive track, the device comprising:
a contact formed of a composite carbon fiber material having at least one layer (150) of carbon fiber elements, wherein the carbon fiber elements within each layer are aligned in substantially the same direction and free ends of at least one layer of carbon fiber elements are adapted to contact said electrically conductive track, **characterised in that** said at least one layer of carbon fiber elements is sandwiched between first and second mats (152,154) formed of nonwoven carbon fibers with a thermoplastic resin coating (162,164) on outer surfaces of said first and second mats.

2. The electrical device according to claim 1, wherein said carbon fiber elements in each layer are bonded together.

3. The electrical device according to claim 2, further comprising a support strip (24) having said electrical contact bonded thereto by a synthetic resin compound.

4. The electrical device according to claim 3, wherein said support strip is electrically conductive.

5. The electrical device according to claim 3, wherein said support strip is bent so as to be L-shaped and said electrical contact is attached to a shorter arm of said L-shaped strip (12).

6. The electrical device according to claim 2, wherein the free ends of said layer of carbon fiber elements are formed in a knuckle shape (16).

7. The electrical device according to claim 2, wherein the free ends of said layer of carbon fiber elements are formed in an angularly pointed shape (20).

8. The electrical device according to claim 2, further comprising support elements arranged on either side of said thermoplastic resin coating on said first and second mats at an end opposite said free ends and being set back from said free ends.

9. The electrical device according to claim 2, further comprising:
fastening means (102, 104, 106) arranged at one end of said electrical contact for holding together said layer of carbon fiber elements and preventing relative movement there among at a holding location, whereby free ends of said electrical contact opposite said one end are moveable relative to one another.

10. The electrical device according to claim 9, wherein the free ends of said layer of carbon fiber elements are formed in a knuckle shape.

11. The electrical device accordingly to claim 9, wherein the free ends of said layer of carbon fiber elements are found in an angularly pointed shape.

12. The electrical device according to claim 2, wherein electrical contact has a first arm portion (74) and a second arm portion (76) spaced apart from and in a same plane as said first arm portion, wherein the carbon fiber elements therein are aligned substantially in the same first direction, and a transition portion (72) connecting respective first ends of said first arm portion and said second arm portion, wherein the carbon fiber elements of said transition portion are substantially aligned with each other in a second direction different from said first direction of said first and second arm portions, wherein second ends of said first and second arm portions opposite said first ends are adapted to contact said electrically conductive tracks.

13. The electrical device accordingly to claim 12, wherein said transition portion is arranged at right angles to said first and second arm portions, so that said second direction is substantially perpendicular to said first direction.

14. The electrical device according to claim 12, wherein said transition portion (60) is semicircular in shape and is coplanar with said first and second arm portions.

15. The electrical device according to claim 2, comprising a plurality of overlying layers (42, 44, 46) of carbon fibers formed as a matrix, wherein the carbon fibers in each of said plurality of layers are aligned so as to be substantially parallel and adjacent layers are aligned so that the carbon fibers therein are substantially nonparallel, wherein an electrically conductive synthetic resin compound binds together said carbon fibers in each layer so that said plurality of overlying layers solidify said electrical contact.

16. The electrical device according to claim 15, wherein said electrical contact is formed having a body portion and first and second arm portions extending therefrom, wherein free ends of said first and second arm portions are adapted to contact the electrically conductive tracks.

17. The electrical device according to claim 16, wherein said free ends are formed in a rake shape.

18. The electrical device according to claim 16, wherein said plurality of overlying layers are coextensive.

19. The electrical device according to claim 16, wherein said first and second arm portions are formed of a single layer of carbon fibers.

20. The electrical device as claimed in claim 1 further comprising:
an electrically conductive carrier (128);
a plurality of layers of carbon fiber elements arranged in overlaying relationship and affixed on said carrier.

21. The electrical device according to claim 20, wherein said carrier is substantially L-shaped and said plurality of layers of carbon fiber elements are affixed to a shorter leg (126) of said L-shaped carrier.

## Patentansprüche

1. Elektrische Vorrichtung zum Übertragen von elektrischen Signalen und für den beweglichen Kontakt mit einer elektrisch leitfähigen Schiene, wobei die Vorrichtung Folgendes umfasst:
einen aus einem Kohlenstofffaser-Verbundmaterial gebildeten Kontakt mit mindestens einer Schicht (150) aus Kohlenstofffaserelementen, wobei die Kohlenstofffaserelemente in jeder Schicht in der im Wesentlichen selben Richtung ausgerichtet sind und freie Enden mindestens einer Schicht von Kohlenstofffaserelementen dazu angepasst sind, die genannte elektrisch leitfähige Schiene zu berühren, **dadurch gekennzeichnet, dass** die genannte mindestens eine Schicht aus Kohlenstofffaserelementen sandwichartig zwischen einer ersten und einer zweiten Matte (152, 154) angeordnet ist, die aus nicht gewebten Kohlenstofffasern mit einer thermoplastischen Harzbeschichtung (162, 164) auf Außenflächen der genannten ersten und der genannten zweiten Matte gebildet sind.

2. Elektrische Vorrichtung nach Anspruch 1, wobei die genannten Kohlenstofffaserelemente in jeder Schicht zusammengeklebt sind.

3. Elektrische Vorrichtung nach Anspruch 2, weiter umfassend einen Stützstreifen (24), an den der genannte elektrische Kontakt mit einer Kunstharzverbindung geklebt ist.

4. Elektrische Vorrichtung nach Anspruch 3, wobei der genannte Stützstreifen elektrisch leitfähig ist.

5. Elektrische Vorrichtung nach Anspruch 3, wobei der genannte Stützstreifen gebogen ist, so dass er L-förmig ist und der genannte elektrische Kontakt an einem kürzeren Arm des genannten L-förmigen Streifens (12) angebracht ist.

6. Elektrische Vorrichtung nach Anspruch 2, wobei die freien Enden der genannten Schicht aus Kohlenstofffaserelementen in einer Knöchelform (16) ausgebildet sind.

7. Elektrische Vorrichtung nach Anspruch 2, wobei die freien Enden der genannten Schicht aus Kohlenstofffaserelementen in einer eckigen spitzen Form (20) ausgebildet sind.

8. Elektrische Vorrichtung nach Anspruch 2, weiter umfassend Stützelemente, die auf beiden Seiten der genannten thermoplastischen Harzbeschichtung auf der genannten ersten und der genannten zweiten Matte an einem den genannten freien Enden gegenüberliegenden Ende angeordnet sind und von den genannten freien Enden zurückgesetzt sind.

9. Elektrische Vorrichtung nach Anspruch 2, weiter umfassend:
Befestigungsmittel (102, 104, 106), die an einem Ende des genannten elektrischen Kontakts angeordnet sind, um die genannte Schicht aus Kohlenstofffaserelementen zusammenzuhalten und die Relativbewegung dazwischen an einem Halteort zu verhindern, wobei freie Enden des genannten elektrischen Kontakts gegenüber von dem genannten einen Ende relativ zueinander beweglich sind.

10. Elektrische Vorrichtung nach Anspruch 9, wobei die freien Enden der genannten Schicht aus Kohlenstofffaserelementen in einer Knöchelform ausgebildet sind.

11. Elektrische Vorrichtung nach Anspruch 9, wobei die freien Enden der genannten Schicht aus Kohlenstofffaserelementen in einer eckigen spitzen Form gefunden sind.

12. Elektrische Vorrichtung nach Anspruch 2, wobei der elektrische Kontakt einen ersten Armabschnitt (74) hat und einen zweiten Armabschnitt (76) hat, der von dem genannten ersten Armabschnitt beabstandet ist und mit diesem in einer Ebene liegt, wobei die Kohlenstofffaserelemente darin im Wesentlichen in der selben ersten Richtung ausgerichtet sind und ein Übergangsabschnitt (72) jeweilige erste Enden des genannten ersten und des genannten zweiten Armabschnitts verbindet, wobei die Kohlenstofffaserelemente des genannten Übergangsabschnitts im Wesentlichen in einer zweiten Richtung, die von der genannten ersten Richtung des genannten ersten und des genannten zweiten Armabschnitts verschieden ist, miteinander ausgerichtet sind, wobei, den genannten ersten Enden gegenüberliegende zweite Enden des genannten ersten und des genannten zweiten Armabschnitts dazu angepasst sind, die genannten elektrisch leitfähigen Schienen zu berühren.

13. Elektrische Vorrichtung nach Anspruch 12, wobei der genannte Übergangsabschnitt rechtwinklig zum genannten ersten und zum genannten zweiten Armabschnitt angeordnet ist, so dass die genannte zweite Richtung im Wesentlichen senkrecht zu genannten ersten Richtung ist.

14. Elektrische Vorrichtung nach Anspruch 12, wobei der genannte Übergangsabschnitt (60) halbkreisförmig ist und mit dem genannten ersten und dem genannten zweiten Armabschnitt koplanar ist.

15. Elektrische Vorrichtung nach Anspruch 2, umfassend eine Vielzahl übereinander liegender Schichten (42, 44, 46) aus Kohlenstofffasern, die als eine Matrix ausgebildet sind, wobei die Kohlenstofffasern in jeder der genannten Vielzahl von Schichten so ausgerichtet sind, dass sie im Wesentlichen parallel sind und benachbarte Schichten so ausgerichtet sind, dass die Kohlenstofffasern darin im Wesentlichen nicht parallel sind, wobei eine elektrisch leitfähige Kunstharzverbindung die genannten Kohlenstofffasern in jeder Schicht verbindet, so dass die genannte Vielzahl übereinander liegender Schichten den genannten elektrischen Kontakt verfestigen.

16. Elektrische Vorrichtung nach Anspruch 15, wobei der genannte elektrische Kontakt mit einem Körperabschnitt und einem ersten und einem zweiten, sich davon erstreckenden Armabschnitt gebildet ist, wobei freie Enden des genannten ersten und des genannten zweiten Armabschnitts dazu angepasst sind, die elektrisch leitfähigen Schienen zu berühren.

17. Elektrische Vorrichtung nach Anspruch 16, wobei die genannten freien Enden in einer Rechenform ausgebildet sind.

18. Elektrische Vorrichtung nach Anspruch 16, wobei die genannte Vielzahl übereinander liegender Schichten längengleich sind.

19. Elektrische Vorrichtung nach Anspruch 16, wobei der genannte erste und der genannte zweite Armabschnitt aus einer einzigen Schicht aus Kohlenstofffasern gebildet sind.

20. Elektrische Vorrichtung nach Anspruch 1, die weiter Folgendes umfasst:
einen elektrisch leitfähigen Träger (128);
eine Vielzahl von Schichten aus Kohlenstofffaserelementen, die in übereinander liegender Beziehung angeordnet und auf dem Träger befestigt sind.

21. Elektrische Vorrichtung nach Anspruch 20, wobei der genannte Träger im Wesentlichen L-förmig ist und die genannte Vielzahl von Schichten aus Kohlenstofffaserelementen an einem kürzeren Bein (126) des genannten L-förmigen Trägers befestigt sind.

## Revendications

1. Dispositif électrique pour émettre des signaux électriques et établir un contact mobile avec une piste électriquement conductrice, le dispositif comprenant :
un contact formé d'une matière de fibre de carbone composite ayant au moins une couche (150) d'éléments de fibre de carbone, dans lequel les éléments de fibre de carbone dans chaque couche sont alignés essentiellement dans le même sens et les extrémités libres d'au moins une couche d'éléments de fibre de carbone sont adaptées pour faire contact avec ladite piste électriquement conductrice, **caractérisé en ce que** ladite au moins une couche d'éléments de fibre de carbone est prise en sandwich entre des premier et deuxième tapis (152, 154) formés de fibres de carbone non tissées avec un revêtement de résine thermoplastique (162, 164) sur les surfaces externes desdits premier et deuxième tapis.

2. Dispositif électrique selon la revendication 1, dans lequel lesdits éléments de fibre de carbone dans chaque couche sont collés ensemble.

3. Dispositif électrique selon la revendication 2, comprenant en outre une barrette de support (24) sur laquelle est collé ledit contact électrique par un composé de résine synthétique.

4. Dispositif électrique selon la revendication 3, dans lequel ladite barrette de support est électriquement conductrice.

5. Dispositif électrique selon la revendication 3, dans lequel ladite barrette de support est pliée de façon à avoir une forme de L et ledit contact électrique est fixé à un bras plus court de ladite barrette en forme de L (12).

6. Dispositif électrique selon la revendication 2, dans lequel les extrémités libres de ladite couche d'éléments de fibre de carbone sont formées en forme d'articulation (16).

7. Dispositif électrique selon la revendication 2, dans lequel les extrémités libres de ladite couche d'éléments de fibre de carbone sont formées en une forme angulairement pointue (20).

8. Dispositif électrique selon la revendication 2, comprenant en outre des éléments de support disposés de chaque côté dudit revêtement de résine thermoplastique sur lesdits premier et deuxième tapis au niveau d'une extrémité opposée auxdites extrémités libres et étant en retrait par rapport auxdites extrémités libres.

9. Dispositif électrique selon la revendication 2, comprenant en outre :
des moyens de fixation (102, 104, 106) disposés au niveau d'une extrémité dudit contact électrique pour maintenir ensemble ladite couche d'éléments de fibre de carbone et empêcher un mouvement relatif parmi eux au niveau d'une position de maintien, de telle sorte que les extrémités libres dudit contact électrique opposées à ladite une extrémité soient mobiles les unes par rapport aux autres.

10. Dispositif électrique selon la revendication 9, dans lequel les extrémités libres de ladite couche d'éléments de fibre de carbone sont formées en forme d'articulation.

11. Dispositif électrique selon la revendication 9, dans lequel les extrémités libres de ladite couche d'éléments de fibre de carbone se trouvent dans une forme angulairement pointue.

12. Dispositif électrique selon la revendication 2, dans lequel le contact électrique a une première partie de bras (74) et une deuxième partie de bras (76) espacée de ladite première partie de bras et située dans le même plan que celle-ci, dans lequel les éléments de fibre de carbone s'y trouvant sont sensiblement alignés dans le même premier sens, et une partie de transition (72) connectant des premières extrémités respectives de ladite première partie de bras et de ladite deuxième partie de bras, dans lequel les éléments de fibre de carbone de ladite partie de transition sont sensiblement alignés les uns avec les autres dans un deuxième sens différent dudit premier sens desdites première et deuxième parties de bras, dans lequel lesdites deuxièmes extrémités desdites première et deuxième parties de bras opposées auxdites premières extrémités sont adaptées pour faire contact avec lesdites pistes électriquement conductrices.

13. Dispositif électrique selon la revendication 12, dans lequel ladite partie de transition est agencée en angle droit avec lesdites première et deuxième parties de bras, de telle sorte que ledit deuxième sens soit sensiblement perpendiculaire audit premier sens.

14. Dispositif électrique selon la revendication 12, dans lequel ladite partie de transition (60) est de forme semicirculaire et est coplanaire avec lesdites première et deuxième parties de bras.

15. Dispositif électrique selon la revendication 2, comprenant une pluralité de couches sus-jacentes (42, 44, 46) de fibres de carbone formées en matrice, dans lequel les fibres de carbone dans chacune de ladite pluralité de couches sont alignées de façon à être sensiblement parallèles et les couches adjacentes sont alignées de telle sorte que les fibres de carbones s'y trouvant soient sensiblement non parallèles, dans lequel un composé de résine synthétique électriquement conducteur lie ensemble les fibres de carbone dans chaque couche de telle sorte que ladite pluralité de couches sus-jacentes solidifie ledit contact électrique.

16. Dispositif électrique selon la revendication 15, dans lequel ledit contact électrique est formé avec une partie de corps et lesdites première et deuxième parties de bras s'étendant depuis celui-ci, dans lequel les extrémités libres desdites première et deuxième parties de bras sont adaptées pour faire contact avec les pistes électriquement conductrices.

17. Dispositif électrique selon la revendication 16, dans lequel lesdites extrémités libres sont formées en forme de râteau.

18. Dispositif électrique selon la revendication 16, dans lequel ladite pluralité de couches sus-jacentes s'étend dans le même sens.

19. Dispositif électrique selon la revendication 16, dans lequel lesdites première et deuxième parties de bras sont formées en une seule couche de fibres de carbone.

20. Dispositif électrique selon la revendication 1, comprenant en outre :
un support électriquement conducteur (128) ;
une pluralité de couches d'éléments de fibre de carbone agencée en une relation sus-jacente et fixée sur ledit support.

21. Dispositif électrique selon la revendication 20, dans lequel ledit support a sensiblement une forme de L et ladite pluralité de couches d'éléments de fibre de carbone est fixée à une jambe plus courte (126) dudit support en forme de L.
